

# United States Patent [19]

Amidon et al.

[11] 4,078,927

[45] Mar. 14, 1978

[54] PHOTOCONDUCTIVE PRINTING MASTER

[75] Inventors: Alan B. Amidon; Joseph Mammino, both of Penfield, N.Y.

[73] Assignee: Xerox Corporation, Stamford, Conn.

[21] Appl. No.: 424,497

[22] Filed: Dec. 13, 1973

[51] Int. Cl.<sup>2</sup> ..... G03G 5/04; G03F 7/02

[52] U.S. Cl. ..... 96/1 R; 96/1.5 R; 96/33; 101/356; 101/357; 101/454; 101/456; 101/457; 101/460; 101/462; 101/465

[58] Field of Search ..... 96/1.5, 33; 260/46.5; 101/356, 357, 454, 456, 457, 460, 462, 465

## [56] References Cited

### U.S. PATENT DOCUMENTS

|           |         |         |       |        |
|-----------|---------|---------|-------|--------|
| 3,408,186 | 10/1968 | Mammino | ..... | 96/1.5 |
| 3,408,187 | 10/1968 | Mammino | ..... | 96/1.5 |
| 3,408,190 | 10/1968 | Mammino | ..... | 96/1.5 |

|           |         |                      |            |
|-----------|---------|----------------------|------------|
| 3,554,125 | 1/1971  | Van Dorn et al. .... | 96/1.5     |
| 3,606,922 | 9/1971  | Doggett .....        | 101/457    |
| 3,775,115 | 11/1973 | Sorkin et al. ....   | 96/33      |
| 3,804,620 | 4/1974  | Wells .....          | 96/1.5     |
| 3,819,744 | 6/1974  | Büchner et al. ....  | 260/46.5 R |
| 3,820,984 | 6/1974  | Gundlach .....       | 96/1.5     |
| 3,821,325 | 6/1974  | Merritt et al. ....  | 260/46.5 R |
| 3,859,090 | 1/1975  | Yoerger et al. ....  | 96/1.5     |
| 3,861,915 | 1/1975  | Cawley .....         | 96/1.5     |
| 4,030,416 | 6/1977  | Schank .....         | 101/450    |

Primary Examiner—Edward C. Kimlin

Attorney, Agent, or Firm—James J. Ralabate; James P. O'Sullivan; Gaetano D. Maccarone

## [57] ABSTRACT

A planographic printing master comprising an ink releasing photoconductive insulating layer and an ink receptive particulate image pattern.

3 Claims, No Drawings

## PHOTOCONDUCTIVE PRINTING MASTER

## BACKGROUND OF THE INVENTION

## 1. Field of the Invention

This invention relates to planographic printing masters prepared by electrostatographic techniques. More specifically, this invention concerns photoconductive printing masters which are especially suitable for use in direct and offset lithographic printing processes.

## 2. Description of the Prior Art

Conventional printing processes can generally be classified in the following categories: (a) relief printing; (b) intaglio printing (c) planographic printing; and (d) porous printing. In relief printing the master or "image carrier" comprises elevated and depressed regions wherein the printed image is prepared by transfer of ink from the elevated areas of the master to the receiving sheet. The reverse situation is found to exist in intaglio printing systems wherein the printing areas of the image carrier are the depressions within the surface of the master and the elevated regions now provide the background for said image. In planographic printing systems, the printing and background regions of the printing master are on substantially the same plane. Porous printing or screen printing processes are distinct from the above systems in two major respects; holes in the screen provide the image areas of the master and the inking of the screen is a part of the image transfer process.

Planographic printing systems are further subdivided into four distinct printing methods. These systems include stone lithography, direct lithography, offset lithography, and collotype. Since the printing and non-printing areas of the lithographic master are located on substantially the same plane, problems are encountered in lithographic printing which are not experienced in other types of printing systems. The major consideration is the selective inking of the imaged areas of the printing plate while at the same time avoiding the transfer of ink to the nonimaged or background areas of the printing plate. This problem can be overcome by treating the background areas with an ink releasing material. After each successive printing sequence, this ink releasing capability of the non-printing areas must be refreshed by what is commonly referred to in the printing art as "dampening". Dampening comprises the treatment of these nonimaged areas with a so-called "fountain solution" containing essentially water or a mixture of water and alcohol (e.g., monohydric or polyhydric alcohols). Since the printing inks generally used in lithography are greasy, they are repelled by the relatively hydrophilic non-imaged areas whereas they are attracted to the relatively oleophilic imaged areas of the master. It is critical that the nonprinting areas remain receptive to the dampening solution and nonreceptive of the printing ink. It is also equally critical that the printing areas of the master remain receptive to ink and repellent to the dampening solution. With the exception of collotype printing systems all lithographic printing processes require dampening and inking for each printing cycle.

This periodic dampening of the printing master has been known to result in "flow back" of fountain solution into the train of ink rollers during the course of a printing run, thereby, causing emulsification of the ink on these rollers. Another problem inherent in the periodic dampening of the printing master is the "carry out"

of fountain solution from such plates to the transfer sheet. Wetting of the transfer sheet with such fountain solutions can cause curling of the sheet, thus, making registration more difficult in the event that such sheet must undergo multiple trips through the press, as is often required in color printing.

The most popular of the planographic printing systems, (based upon commercial considerations), are "direct" and "off-set" lithography. In direct lithography, 10 the ink image is transferred from the printing master directly to a receiving sheet. Offset lithography, on the other hand, involves transfer of the ink image from the lithographic master to a "blanket" or an "impression cylinder" which in turn conveys the ink image to a receiving sheet. While it is apparent that direct lithography provides a simpler printing system due to the absence of an intermediate transfer step, the presence of such a transfer medium does serve a highly desirable function in that it minimizes the "carry out" of a fountain solution from the printing master to the transfer sheet, thus, avoiding wetting of such sheets with fountain solution. The resilient nature of this blanket also enhances transfer image quality and minimizes abrasion of the image pattern on the master.

Until relatively recently, all lithographic printing systems have required some periodic dampening of the printing master between printing cycles in order to renew the ink repellency of the non-printing areas of the lithographic master. A number of lithographic printing

30 systems have been disclosed which reportedly eliminate the need for such periodic dampening. These systems, hereinafter referred to as "waterless lithographic printing systems", base their reported success upon the discovery that certain materials (described as "adhesive" 35 materials) have surface characteristics which defy acceptance of ink from an inking roller and yet are capable of undergoing selective modification (photomechanical or electrical etching) so as to render such modified areas ink receptive, U.S. Pat. No. 3,511,178.

40 More recently, a waterless lithographic printing system has been disclosed wherein an ink receptive image pattern is formed on an adhesive substrate by conventional electrostatographic imaging methods, German patent application OLS P 22 34 692.5, published Jan. 25, 1973. According to this publication, a photoconductive layer is overcoated with a thin film of adhesive material and the resulting structure charged and imaged in accord with standard electrostatographic techniques. The latent image thus formed on the adhesive surface of the 45 structure is rendered visible by development with toner particles which upon fusion to this adhesive layer provide ink receptive characters on this ink releasing background. Other embodiments described in this publication include preparation of photoconductive binder 50 layers wherein the ink releasing (adhesive) materials serve as a binder for a variety of photoconductive pigments (e.g. zinc oxide or anthracene). All of the resulting lithographic masters prepared in compliance with the teachings of this disclosure are reportedly useful in 55 waterless lithographic printing systems and possess good resistance to image breakdown.

60 The principal reasons for the reported success of the above systems apparently reside in the surface characteristics of the adhesive material making up the image carrier. The extent to which such image carriers retain their ink releasing properties is dependent upon the maintenance of such favorable surface characteristics. The incorporation of sufficient quantities of photocon-

ductive pigments within such adhesive materials to render the resulting binder layer photoconductive can, however, result in adverse alteration in the ink releasing properties of such films. This is to be expected since as the concentration of such pigment in the binder increases, the composite layer begins to progressively take on the surface characteristics of the non-adhesive pigments incorporated therein.

It is, therefore, the principal object of this invention to provide a photoconductive lithographic printing master which does not suffer from the deficiencies experienced in such binder layer systems. 10

Accordingly, it is the object of this invention to provide a photoconductive lithographic printing master suitable for use in both offset and direct lithographic printing systems. 15

More specifically, it is the principal object of this invention to provide a photoconductive lithographic printing master wherein the ink receptive toner image is firmly adherent to the ink releasing substrate. 20

It is another object of this invention to provide a photoconductive lithographic printing master which can be prepared by standard electrostatographic techniques. 25

#### SUMMARY OF THE INVENTION

The above and related objects are realized by providing a planographic printing master comprising a conductive substrate having operatively disposed in relation thereto an ink releasing photoconductive insulating layer comprising a block copolymer consisting essentially of polymeric segments from a siloxane monomer and segments from a polymer selected from the group consisting of addition polymers and polycondensates wherein said addition polymers segments and said polycondensates polymer segments contain aromatic and/or heterocyclic constituents either appended from or integrated within the polymer backbone. These aromatic and/or heterocyclic constituents should be capable of providing said polymers with sites capable of (i) an electron donor function, (ii) an electron acceptor function or (iii) both an electron donor and an electron acceptor function. In those polymer systems wherein the aromatic and/or heterocyclic constituent is only capable of performing a single function, namely that of an electron acceptor or an electron donor, sufficient activator molecules are added to the block copolymer in preparation of the ink releasing layer to render said layer photoresponsive to visible light. Such activator molecules are optional where the aromatic and/or heterocyclic constituent is difunctional, namely that is capable of undergoing a charge transfer transition within the structural unit containing such constituent or capable of interaction with other monofunctional or difunctional sites on adjacent segments of the polymer. Especially preferred ink releasing photoconductive insulating layers which are useful in the preparation of the planographic printing masters of this invention comprise block copolymers of poly(dimethylsiloxane) and poly( $\alpha$ -methyl styrene) which have been sensitized by 40 the addition of a strong electron acceptor. 60

#### DESCRIPTION OF THE INVENTION INCLUDING PREFERRED EMBODIMENTS

The photoconductive imaging layer of the lithographic master of this invention is prepared by forming a film from (1) a block copolymer containing polymeric segments from a siloxane monomer and polymeric seg- 65

ments from a non-siloxane monomer and (2) activator compounds, where appropriate. The quantity of polymeric materials deposited on the substrate should be sufficient to provide a dry film thickness in the range of from about 0.1 to about 100 microns.

The siloxane segment (hereinafter also referred to as the "soft segment") of the block copolymer comprises repeating units of organo-functional siloxanes having the following structural formula:



wherein

R and R' are independently selected from alkyl of 1 to 4 carbon atoms, halogenated alkyl of 1 to 4 carbon atoms or nitrile substituted alkyl of 1 to 3 carbon atoms; and

n is at least 25.

The average molecular weight of such soft segments of the block copolymer generally are in excess of 2000 and preferably in excess of  $10^4$ . Organo-functional siloxanes which are suitable for use in such block copolymers are generally readily available commercially or can be prepared by techniques and with apparatus disclosed in the technical literature. Especially preferred organo-functional siloxanes which can be used in preparation of the lithographic masters of this invention include poly(methylsiloxane), poly(dimethylsiloxane), poly (ethylsiloxane), and poly(diethylsiloxane). Although, the literature discloses that some aromatic substitution of the siloxane segment of the adhesive layer can be tolerated in a waterless lithographic printing environment (U.S. Pat. No. 3,511,178), such aromaticity is to be avoided since it can adversely alter the ink releasing properties of such siloxane polymers.

The non-siloxane segments of the block copolymer (hereinafter also referred to as the "hard segments" of the copolymer) can be prepared from any one or combination of addition polymers and polycondensates having aromatic and/or heterocyclic constituents. Of course, the greater the degree of aromatic and/or heterocyclic functionality within the polymer segment, the greater the likelihood of charge transfer interaction with activator molecules and the more favorable the charge carrier transport capability of the polymer. In the preferred embodiments of this invention, each structural unit of the hard segments of the block copolymer has at least one aromatic and/or heterocyclic constituent. Typical of the non-siloxane polymers which are suitable for use in such block copolymers include poly(styrene); poly( $\alpha$ -methylstyrene); poly(N-vinylcarbazole); poly(carbonate) resins comprising recurring units of the formula:



wherein



In an alternative embodiment of this invention, a film of this block copolymer can also contain very small amounts (from about 1 to 10 weight percent based upon the concentration of hard segments of the block copolymer) of photoconductive pigments having a range of spectral response beyond the range of substantial spectral response of the non-siloxane segments of the block copolymer. The principal advantage of such a structure is that it provides a system in which it is possible to separate carrier generation (photoconductive pigment) and transport (block copolymer) functions within the film when the image information is only activating of the carrier generation species within the layer. Similar results are obtained where the image carrier comprises a composite structure having a layer of block copolymer superimposed over a photoconductive insulating layer.

An adhesive polymeric composition of the type previously described can be formed on a conductive (preferably flexible) substrate by any of the techniques traditionally used in the film casting or the coating arts (e.g. dip, draw or spray coating). The dry film thickness of such films can range anywhere from about 0.1 to about 100 microns and preferably from about 2 to about 50 microns; film thickness generally being dictated by durability requirements of the master and the amount of deformation such films undergo during inking and transfer. Typical of the substrates which are satisfactory for fabrication of photoconductive printing masters of this invention include aluminum; chromium; metallized plastic films; metal coated plastic films (e.g. aluminized Mylar); and conductive glass plates (e.g. NESA glass). Subsequent to forming a photoconductive film of the desired thickness of the conductive substrate, the film is allowed to dry until substantially free of residual solvents used in its fabrication. The imaging layer of the resulting member is thereafter sensitized by charging with a corotron of the appropriate polarity; image information projected onto this sensitized imaging surface at a wavelength capable of activating the carrier generating centers of said imaging layer; and the latent image thus produced developed with thermoplastic toner particles. In the event that carrier generation and transport functions are performed by separate components of the imaging layer, the polarity of the sensitizing charge and the wavelength at which the image information is projected onto said sensitized layer must be selected so as to provide for rapid and substantially complete discharge of the charge in the light struck areas on said sensitized layer.

The ink receptive toner used in development of the latent electrostatic image can be almost virtually any thermoplastic material which is both compatible with electrostatographic imaging techniques and which upon fusion to the photoconductive imaging layer provides an ink receptive image pattern. With regard to this latter requirement, it is generally preferable to select materials which are chemically similar to the hard segments of the block copolymer used in preparation of the ink releasing layer results in better adhesion of the image to said layer. Such enhanced adhesion is highly desirable in order to avoid the type of image breakdown which can occur during the use of such imaged member in direct and offset lithographic printing processes. Especially preferred thermoplastic toner materials which satisfy the above requirements are toners containing polymers of styrene and substituted styrene and their copolymers.

5 The Examples which follow further define, describe and illustrate preparation of the planographic printing masters of this invention. Techniques and apparatus used in preparation and evaluation of these masters are presumed to be standard or as hereinbefore described. Parts and percentages appearing in such Examples are by weight unless otherwise stipulated.

#### EXAMPLE I

10 A planographic printing master is prepared by solvent casting a chloroform dispersion of 100 parts by weight of a block copolymer of poly(dimethylsiloxane)/poly( $\alpha$ -methyl styrene) — relative mole ratio 60:40 — and 60 parts by weight 2,4,7-trinitro-9-fluorenone on a ball grained flexible aluminum plate. The amount of dispersion transferred to said plate is sufficient to form a layer having a dry film thickness of about 50 microns. Following evaporation of residual chloroform from said layer, the resulting plate is charged in the dark to a positive potential of about 600 volts in a Xerox Model D processor and subsequently exposed through a Xerox #4 camera at  $f$ 16 for 12 seconds. The source of illumination of said image is a tungsten lamp. The latent electrostatic image thus formed on the plate is developed by cascading a developer composition comprising a poly(styrene-cobutylmethacrylate) toner. The toner image is then fused to the plate with a radiant fuser. The resulting image carrier is inserted in a standard offset lithographic press and the press run without periodic dampening between each printing cycle. The ink used in the lithographic press is available from Pope & Grey Division of Martin Marietta Corporation, Clifton, New Jersey (Pope & Grey #2441 Lithographic Ink). After about 500 prints have been prepared from this lithographic master, both the prints and the master are examined. The particulate image pattern on the lithographic master appears to be intact and the background areas of the prints have remained clean throughout the entire printing run.

#### EXAMPLE II-V

15 The procedures of Example I are repeated except the ink releasing photoconductive insulating layer is cast from a solution comprising 100 parts by weight of block copolymer and 5 parts by weight photoconductive pigment. The plate thus prepared is sensitized as previously described, however, the wavelength of the source of illumination of the image pattern is controlled with the appropriate band pass filter so as to correspond to the wavelength of maximum photoresponse of the photoconductive pigment. The table which follows provides a list of pigments which can be incorporated into the above block copolymer and the appropriate wavelength used in illumination of the image information.

20 TABLE I

| EXAMPLE | NO. | PIGMENT                     | WAVELENGTH OF PEAK PHOTORESPONSE |
|---------|-----|-----------------------------|----------------------------------|
| II      |     | cadmium sulfide             | 450 - 500 millimicrons           |
| III     |     | cadmium sulfoselenides      | 640 millimicrons                 |
| IV      |     | x-metal free phthalocyanine | 625 millimicrons                 |
| V       |     | selenium                    | 420 millimicrons                 |

25 60 65 What is claimed is:

1. A photoconductive planographic printing master comprising:
  - (a) a conductive substrate;

- (b) a photoconductive ink releasing layer operatively disposed in relation to said substrate, said layer comprising 2,4,7-trinitro-9-fluorenone and a block copolymer of soft poly(dimethylsiloxane) segments and hard poly( $\alpha$ -methylstyrene) segments, the relative weight ratio of hard polymer segments to soft polymer segments in said copolymer being in the range of from about 75:25 to about 5:95; and
- (c) an ink receptive image pattern affixed to the surface of said photoconductive layer, said pattern comprising a thermoplastic polymeric material

including styrene and/or substituted styrene segments.

2. The photoconductive planographic printing master of claim, 1 wherein the relative weight ratio of hard polymer segments to soft polymer segments is in the range of from about 25:75 to about 5:95.

3. The photoconductive planographic printing master of claim 1, wherein the ink releasing layer contains from about 1 to about 10 weight percent photoconductive pigment having a range of spectral response beyond the range of photoresponsiveness of the block copolymer.

\* \* \* \* \*

15

20

25

30

35

40

45

50

55

60

65